

Dec. 28, 1954

E. H. LAND

2,698,237

PHOTOGRAPHIC SILVER HALIDE TRANSFER PRODUCT AND PROCESS

Filed Aug. 16, 1954



FIG. 1



FIG. 2



FIG. 3

INVENTOR  
*Edwin H. Land*  
BY  
*Brown and McRuerka*

ATTORNEYS

1

2,698,237

## PHOTOGRAPHIC SILVER HALIDE TRANSFER PRODUCT AND PROCESS

Edwin H. Land, Cambridge, Mass., assignor to Polaroid Corporation, Cambridge, Mass., a corporation of Delaware

Application August 16, 1954, Serial No. 449,995

31 Claims. (Cl. 95—8)

This invention relates to photographic products and processes and more particularly to transfer processes wherein a latent image in a silver halide emulsion is developed and wherein a soluble silver complex obtained by reaction with the undeveloped silver halide of said emulsion is transferred from said emulsion and the silver thereof is precipitated in another layer to form a positive print, and to products useful as print-receiving elements in said processes.

This application is a continuation-in-part of my copending application Serial No. 164,908, filed May 29, 1950, for Photographic Silver Halide Transfer Product and Process, now abandoned, which, in turn, is a continuation-in-part of my copending application Serial No. 727,385, filed February 8, 1947 for Photographic Product and Process.

One object of the present invention is to provide a transfer process of the foregoing type and products for use in said process whereby there are produced positive prints of good quality and stability from silver halide emulsions of high speed.

Another object of the present invention is to provide an improved product particularly useful in the foregoing transfer processes as the print-receiving element, said product comprising a novel silver precipitating layer adjacent one surface thereof, which layer serves to effect a controlled precipitation of the silver from the soluble silver complex and also acts to receive and suitably aggregate the precipitated silver to produce dense positive images of excellent pictorial quality. More specifically, it is an object of the present invention to provide in a product of the foregoing character a silver precipitating layer comprising particles of silica in which the silver precipitating agent is suitably supported.

Still another object of the present invention is to provide a novel print-receiving element which also includes materials for greatly improving the stability of the positive silver print formed in said element.

Other objects of the invention will in part be obvious and will in part appear hereinafter.

The invention accordingly comprises the several steps and relation and order of one or more of such steps with respect to each of the others, and the product possessing the features, properties and the relation of elements which are exemplified in the following detailed disclosure, and the scope of the application of which will be indicated in the claims.

For a fuller understanding of the nature and objects of the invention, reference should be had to the following detailed description taken in connection with the accompanying drawings wherein:

Figure 1 is a diagrammatic enlarged sectional view illustrating the association of elements during one stage of the performance of a transfer process and showing as one of the elements an embodiment of the novel product of the present invention, the thicknesses of the various materials being exaggerated;

Fig. 2 is a perspective view, with parts broken away, of one form of print-receiving element upon which containers of the processing agent are so positioned as to be capable of distributing their contents between the surface of the print-receiving element and a photosensitive element; and

Fig. 3 is a view similar to Fig. 1 of another form of the print-receiving element of the invention.

The present invention comprehends improved processes and products of the type whereby a positive print is ob-

2

tained in a single step by suitably treating a silver halide emulsion containing a latent image with a uniformly applied layer of processing liquid. Preferably, the processing liquid is in a viscous condition and is spread in a liquid film between the photosensitive element comprising the silver halide emulsion and a print-receiving element comprising a suitable silver precipitating layer. The liquid develops the latent image in the emulsion and forms a soluble silver complex, e. g., a thiosulfate or a thiocyanate, with undeveloped silver halide. This soluble silver complex is at least in part transported in the direction of the print-receiving element and the silver thereof is largely precipitated in the silver precipitating layer of said element to form a positive image in silver.

It has been proposed to use in the formation of the silver transfer prints by the foregoing process certain compounds and elements whose presence during the process has a desirable effect on the amount and character of the silver precipitated during image formation. For this purpose, such materials as, for example, the metallic sulfides and selenides, thiooxalates, and thioacetamides have been disclosed in my U. S. Patent No. 2,647,056, issued July 28, 1953 for One-Step Photographic Transfer Process. Other precipitating agents have been proposed such, for example, as colloidal silver.

According to the present invention, the precipitation and aggregation of silver obtained by using silver precipitating agents, including the above-mentioned materials, is very greatly improved and expedited by providing in the print-receiving element as a dispersing medium or matrix for said agents a layer formed primarily of particles of silica.

The particles are small enough so that when laid down as a thin layer they present a continuous surface to the naked eye rather than a skeletal or porous structure. To this end the particles are submacroscopic in size, i. e., small enough to be indistinguishable as discrete or separate particles by the naked eye.

Preferably they are so small as to approach or be of colloidal size but are nevertheless discrete particles rather than integral parts of a single continuous coalesced mass. Thus, the matrix of the present invention is formed of definite particles which are essentially silica and which are sufficiently small to be indistinguishable as particles by the naked eye when formed into a layer and whose minimum average size is of colloidal rather than of molecular proportions. The essentially pure forms of silica such as the silica aerogel available under the trade name "Santocel C" or the solid content of the hydrated silica dispersions available under the trade names "Ludox" and "Syton" give best results. However, it is possible to use highly pulverized forms of the less pure silicas such, for example, as those obtained from natural sources, provided, however, that these materials have a high silica content of approximately 70% or greater by weight and the particles thereof are submacroscopic in size. Examples of such materials are the silicas derived from diatomites variously known as diatomaceous earth, kieselguhr and infusorial earth. Also useful, when pulverized to particles small enough in size, is powdered glass. However, the preferred materials are silicas whose solid content comprises of the order of 97% or more of  $\text{SiO}_2$ .

The novel silver precipitating layer including the silica and the silver precipitating agent is preferably applied to a suitable support, for example by being coated on the support in the form of a suspension which contains a substantially greater amount of the silica than of the precipitating agent. The support may be formed of a non-siliceous material such as paper, regenerated cellulose, polyvinyl alcohol, cellulose ethers such as methyl cellulose, ethyl cellulose, or their derivatives, such as sodium carboxymethyl cellulose and hydroxyethyl cellulose, and other natural and synthetic gums and resins which will form continuous films and which are relatively stable, mechanically, in the presence of water and alkali. These supporting sheets are opaque when a reflection print is desired and transparent when a transparency is desired.

Suitable as silver precipitating agents are the metallic sulfides and selenides, these terms being understood to include the selenosulfides, the polysulfides, and the poly-selenides. Preferred in this group are the so-called

United States Patent Office

"heavy metal" sulfides, e. g., of zinc, chromium, gallium, iron, cadmium, cobalt, nickel, lead, antimony, bismuth, silver, cerium, arsenic, copper; and the "heavy metal" selenides, e. g., of lead, zinc, antimony and nickel. For best results it is preferred to employ the sulfides whose solubility products in an aqueous medium at approximately 20° C. vary between  $10^{-23}$  and  $10^{-30}$  and specifically the salts of zinc, cadmium and lead. Also suitable as precipitating agents are heavy metals such as silver, gold, platinum, palladium and mercury, and in this category the noble metals are preferred and are preferably provided in the matrix as colloidal particles. Also useful as silver precipitating agents are the salts of these heavy metals, preferably the simple inorganic and readily reducible salts such as silver nitrate, gold chloride and gold nitrate. In some instances, the metals are introduced into the matrix as salts and then reduced in situ prior to the use of the reception material in the silver transfer process to give a layer whose silver precipitating agent is the colloidal metal. Where the salts are relatively light- or heat-sensitive, this reduction may be accomplished simply by exposing the silver precipitating layer to diffuse light or to heat. Still other satisfactory silver precipitating agents are certain of the thio compounds, e. g., dithiooxamate and its lead and zinc complexes, potassium dithiooxalate and the lead and nickel complexes thereof and thiocacetamide. The silver precipitating agents as noted above are provided in a highly dispersed condition, preferably as colloidal particles.

In general, the sulfides and selenides of the alkali metals and alkali earth metals such as sodium, potassium, cesium, calcium, barium and magnesium are too soluble to give optimum pictorial quality, although the provision of a silica layer as a vehicle for such precipitating agents greatly improves the results obtained with said agents.

The concentration of the silica in the silver precipitating layer is preferably high enough to give a macroscopically continuous discrete stratum thereof on the surface of the print-receiving element when applied thereto and the silver precipitating agent is present in a very small amount.

It has been determined that further improvements in image quality are obtained when using one or more of the heavy metal sulfides and selenides as silver precipitating agents if the sulfide or selenide ions of the crystals are prevented from wandering or diffusing during precipitation from their original loci in the precipitating layer. In the following discussion of this and other phenomena involving the action of the sulfide and selenide salts, reference will be made to the sulfides alone, but it is to be understood that wherever such reference is made, the same, unless otherwise stated, is generally applicable to the selenides.

To prevent the diffusion and wandering of the sulfide ions, there is preferably included in the silver precipitating layer or closely adjacent thereto at least one metallic salt which is substantially more soluble in the processing agent than the heavy metal sulfide used as the silver precipitating agent and which is irreducible in the processing agent, said more soluble salt having, as its cation, a metal whose ions form sulfides which are difficultly soluble in the processing agent and which give up their sulfide ions to silver by displacement. Accordingly, when such sulfide ions are present, the metal ions of the more soluble salt have the effect of immediately precipitating the sulfide ions from solution.

The special function of this combination of a sulfide, a more soluble metallic salt and a silica will be better understood by considering the new sequence of reactions which takes place when a print-receiving element so constituted is used in a silver halide transfer process involving a silver halide developer and a silver halide solvent, such as sodium thiosulfate. This sequence of reactions is perhaps best described in my article "One-Step Photography" appearing in Section A of the January, 1950 issue of the "Photographic Journal" (British) as follows:

"First: The silver ion in the silver halide of the negative is protected by its environment in the crystalline halide from being reduced, but it prefers the thiosulfate ion as an associate, so the silver halide dissolves.

"Second: The silver ion is now protected from reduction by the thiosulfate complex, but it prefers the sulfide ion as an associate, so that silver sulfide is formed and would be precipitated as such if it were not for the

fact that the sulphide ion—in spite of the insolubility of the crystalline compound—does not protect the silver ion from reduction. Thus, the silver ion has been safely pried loose and transported to a new site where it becomes silver, and the transporting ions are free to carry on their cyclic efforts. Is this then the end? Actually, it is the beginning, for while we have learned how to extract the silver ions from the negative and to precipitate them as reduced silver rapidly, we are just beginning to consider how to build up an acceptable positive from the point of view of appearance (and of course we have not yet considered our problems of stabilizing an image resident in this complicated reagent).

"What we find when we use sulphide ions to release silver ions from the thiosulfate complex is the following gamut of problems:

"(1) Sulphide ions in solution provide so many points of initiation that an enormous number of grains start growing. If these become large the whole picture will be too dense. If they remain small, the picture will be bright yellow (you will recall that the colour of silver colloids depends on the particle size).

"(2) There is a tendency for the grains in the shadows, opposite the unexposed portions of the negative, where much silver is available, to grow larger than the grains in the medium tones, where the available silver concentration is low, producing an unpleasant combination of blue shadows and yellow high lights.

"(3) Some of the sulphide ions migrate into the negative, dropping the concentration in the positive and fogging the negative.

"Thus, having determined how to extract silver ions from the appropriate part of the negative, and how to reduce them to silver atoms, we are still confronted with the problem of how to build these atoms into arrays of the correct diameter for absorbing visible light. We must also achieve adequate constancy in diameter so that high light and shadow are the same hue.

"Since the sulphide ions are the last factor in the chain of events leading to silver precipitation, let us consider how these might be arranged to influence the array of silver atoms. Let us suppose that we can arrange the sulphide ions in clusters, allowing the diameter of the cluster to be that of the mass of silver we seek to build. The actual mass of sulphide ions might then be very low indeed—subject to one vital proviso, namely that as the sulphide ions perform their cyclic function, they are retained within the diameter that we have chosen for the cluster. If we can meet this condition, then we can cause the silver atoms to fill in the volume of the cluster to make our mass of silver of the required density and size. To do all this we must extend the chain of circumstances that we have been following from the negative outward.

"By forming colloidal crystals of heavy metal sulfides which are not reducible generally in or soluble in the developer, and by aggregating these colloidal crystals into galaxies of our chosen diameter, we can arrange the sulphide ions as we desire them. In this new environment the sulphide ion is bound in place until the silver thiosulfate complex touches it. The silver ion—just as it once left the halide ion for the complex—now leaves the complex ion to form the sulphide. The sulphide similarly leaves the metal ion for association with the silver. Then the silver is reduced—but mark you, reduced in situ—reduced at the point where we originally deposited the colloidal particle of metal sulphide. We have started well in building up our mass of silver. But the sulphide ion, now free, is not likely to encounter the metal ion to which it was bound if it escapes from the galaxy and wanders off. We are in danger of reverting to some extent to the problems that occurred with the soluble sulphide. This danger can be avoided by introducing into the positive sheet at the time of manufacture a relatively high concentration of a soluble salt of the same metal that we used in the colloidal sulphide (or indeed of some other metal, providing that its sulphide is more soluble than silver sulphide and is not reducible in, or soluble in, the developer). After the viscous developer is spread, the metal salt in the positive sheet dissolves, and because of the relatively high concentration of these metal ions, the sulphide that is freed at its original site by the reduction of the silver is at once captured before it can leave that site, and reprecipitated as the sulphide of the metal. In this way, the diameter of the

galaxy is maintained in spite of the cyclic use of the sulphide ions. The silver ions are reduced to silver over the same area that we chose for the original galaxy, and the diameter of the mass of silver is such that our image is the colour we predetermined when we prepared the metal-sulphide galaxies.

"One remarkable aspect of pictures made in this way is that the silver in the positive has very high covering power—in the order of five times that of the silver in the negative. Consequently a good positive can be made from a layer of silver halide that is many times thinner than is ordinarily required for a negative. While full thickness negatives can be used for making this new kind of positive, it is impressive to see how thin a layer of negative material suffices. The negative image, when such a thin emulsion is used, is only just visible, yet the positive derived from the same amount of silver is rich and brilliant. Thus, we see that this process provides a type of intensification. Furthermore, since only the surface of the negative is involved, there is gain in speed, and a gain in sharpness both in exposing and printing. Indeed the migration distance for the silver ions going from the negative sheet to the positive image can be extremely small. We have seen that these ions come from very near the surface of the negative, and we can, if we choose, precipitate the silver in the viscous positive layer at the surface of the negative. Thus, the combination of minimized light scattering in the negative, the short migration distance for the silver ions, and the prompt precipitation of them when they reach the positive, results in a process with quite good resolving power. Furthermore, the pictures are by all ordinary standards grainless, because of the way in which the silver is deposited and aggregated." (Underlined words added or modified.)

The silver precipitating agent is dispersed in silica which aids the formation of the aforementioned galaxies, and it is evident, from the foregoing, that the presence of the more soluble salt, which provides the cations for capturing the free sulfide ions, has the effect of maintaining this desirable aggregation of the sulfide ions during the silver precipitation. These more soluble or ion-capturing salts may be the soluble salts of any of the following metals: cadmium, cerium(ous), cobalt(ous), iron, lead, nickel, manganese, thorium and tin. Satisfactory soluble and stable salts of the above metals may be found, for example, among the following groups of salts: the acetates, the nitrates, the borates, the chlorides, the sulfates, the hydroxides, the formates, the citrates and the dithionates. The acetates and nitrates of zinc, cadmium, nickel and lead are preferred. In general, it is also preferable to use the white or lightly colored salts although for certain special purposes the more darkly colored salts can be employed.

One method of providing the print-receiving element with a silver precipitating layer containing the silver precipitating agent, the salts for capturing the sulfide ions and the silica is to form an aqueous dispersion of silica aerogel to which there is added a suitable quantity of one or more of the ion-capturing salts. Thereafter a substantially lesser molar quantity of a soluble sulfide, such as sodium sulfide, is added. The anions of sulfide and the cations of the ion-capturing salt combine to precipitate from the solution relatively insoluble crystals of the sulfide of the metal of the ion-capturing salt, thereby converting a portion of the latter to the sulfide. This produces a dispersion of the insoluble sulfide in the silica sol while leaving in solution the remainder of the ion-capturing salts. The concentration of the latter in the initial solution in relation to the added amount of the soluble sulfide is such as to give in the final layer a substantially greater amount of the ion-capturing salt in proportion to the sulfide.

In another method of forming the silver precipitating layer the sol of silica is first applied as a coating to the print-receiving element and is thereafter impregnated with one or more of the ion-capturing salts by immersing said coated surface of the element in a solution of said salts and permitting the same to dry. Thereafter, by dipping the sheet in a soluble sulfide a predetermined portion of the more soluble salt in the silica layer is converted to give the insoluble sulfide. Some of the ion-capturing salt is also dissolved out of the layer during the second immersion so that allowance for this loss is made in the quantity of the soluble salt which is applied in the first immersion. It may also be desirable to so

form the sulfide in the silver precipitating layer that there is substantially no excess of the more soluble metallic salts in said layer and to provide the more soluble ion-capturing salts in another layer over or under the silver precipitating layer.

It will be readily appreciated that the performance of a photographic processing, which involves the formation of a positive print by means of a single liquid application, without recourse to baths of liquid, is to be greatly desired where this can be accomplished to give a positive print of good pictorial quality from emulsions of high speed as can be had by following the practices described hereinabove. However, because the usual developing solution is a highly alkaline solution containing a developing agent which rapidly oxidizes in an alkaline environment, it will also be appreciated that under normal circumstances this type of liquid processing provides in the print-receiving element a material which, upon exposure to air, tends to form undesirable stains. Unless the print is subjected to a thorough washing, this condition will normally adversely affect with time the quality of an image formed in a print-receiving layer. However, as pointed out in my U. S. Patents No. 2,584,030, issued January 29, 1952, No. 2,635,048, issued April 14, 1953, and No. 2,644,756, issued July 7, 1953, it is possible to avoid this stain by including in the print-receiving layer a substance which substantially eliminates the stain-forming propensity of the developing solution in the print-receiving layer.

It is to be observed that the ion-capturing salts, to which reference has been made hereinabove, may also serve the function of improving the stability of the positive print provided that they possess, in addition to the aforementioned characteristics, the requisites specified in my above-mentioned U. S. Patent No. 2,584,030. For example, if the ion-capturing salt is a salt of a metal which slowly forms insoluble or slightly soluble metallic hydroxides with the hydroxyl ions in the alkaline processing liquid, it will suitably control the alkalinity of the print-receiving element to substantially, if not totally, prevent the formation of undesirable developer stains.

The stabilizing salt should not be a fogging agent and preferably should be white or lightly colored and should give hydroxides which are also white or light in color. It should not decompose in aqueous non-alkaline solutions. For this purpose, the acetates and nitrates, especially of lead, zinc, nickel and cadmium, are preferred. Of the salts hereinabove set out as being satisfactory for preventing the sulfide ions from wandering, all except the hydroxide will function satisfactorily as stabilizing agents. In addition, the soluble salts, for example, of aluminum, may be used to stabilize although they will not serve to trap the wandering sulfide ions.

The use of the novel products of the present invention in the performance of a silver halide transfer process is illustrated diagrammatically in Fig. 1, wherein 10 represents a photosensitive element comprising a support 10a and a photosensitive silver halide emulsion layer 10b, 14 represents a layer of relatively viscous processing agent, and 12 is one embodiment of the novel print-receiving element of the invention upon which a transfer print is obtained by the process. As shown, the print-receiving element 12 comprises a suitable support 12a and a silver precipitating layer 16.

Liquid layer 14 may be obtained by spreading the processing agent, for example, in a manner disclosed in my above-mentioned U. S. Patent No. 2,647,056, and the processing agent may be one of the film-forming processing agents disclosed in said patent. It may comprise, for example, a developing agent such as hydroquinone, an alkali such as sodium hydroxide, a substance, such as sodium thiosulfate, for forming a soluble silver complex with unexposed silver halide, and a high molecular weight film-forming thickening agent such as sodium carboxymethyl cellulose. All these materials are preferably in aqueous solution. These various photographic reagents are preferably contained in solution in the processing liquid prior to the spreading thereof as a layer 14, but they may be in part or wholly added to the processing liquid as it is spread between elements 10 and 12, said reagents being so located on or adjacent the surface of one or both of said elements as to be dissolved by or otherwise interacted with the liquid agent when the latter wets said surface.

The liquid processing agent may be provided for spread-

ing as a layer 14 between elements 10 and 12 by being contained in an elongated rupturable container 20 which, as shown in Fig. 2, has a length at least equal to the transverse dimension of the area of photosensitive element 10 to which the liquid processing agent is to be applied. One or more containers 20 may be attached to one of elements 10 and 12 and, in Fig. 2, two such containers are shown secured to the print-receiving surface of element 12, being spaced apart, lengthwise of said element, a distance equal at least to the length of a single frame of the photosensitive element 10. Said elements 10 and 12 may be connected together so that they can be superposed with the container so positioned that it can release its contents in a film therebetween. The container 20 is preferably inexpensive and disposable and so constructed as to be capable of retaining the liquid processing agent or composition therein for relatively long periods of time without vapor loss or oxidation. One example of a suitable container of this type is formed from a single multilayer sheet of material comprising three laminae. The inner lamina, which provides the inner surface of the container, is formed of a material which is chemically inert to the reagents in the processing agent and which is impervious to the liquid of the agent. One class of materials suitable for this purpose, particularly where the processing agent is an alkaline solution, is the polyvinyl acetals, and of the acetals, polyvinyl butyral is a preferred species. A composition comprising 60% to 72% by weight of polyvinyl butyral, 10% to 23% by weight of nitrocellulose, and approximately 5% by weight of dibutyl sebacate is satisfactory as the inner lamina. The intermediate lamina is preferably impervious to the vapor of the processing agent and is formed, for example, of a metallic foil such as lead or silver foil. The outer or backing lamina is formed of a strong, deformable, relatively inexpensive sheet material such as a kraft paper.

The container 20 is preferably formed by taking the single sheet of three-ply material and folding the same medially at 22, and thereafter securing the end marginal portions 24 and the longitudinal portions 26 of the two folded faces to one another, providing a central space or cavity 28 for containing the processing liquid.

To fill the container it is possible to adhere together the opposite longitudinally extending marginal portions 26 and one of the end marginal portions 24, the container being filled through the other end which is thereafter sealed.

Photosensitive element 10 may be any of the commercially available photosensitive silver halide films, the term "films" being understood to include paper-backed emulsions. The products of the present invention are particularly useful in improving the results obtained when the transfer process is carried out with one of the high-speed photosensitive silver halide emulsions such as the emulsion of the relatively high-speed orthochromatic films, e. g., Eastman Kodak Verichrome film, having an ASA speed rating of 0200 and an ASA exposure index rating in the daylight of 50, and the extremely high-speed panchromatic emulsions, e. g., Eastman Kodak Super XX Pan having an ASA speed rating of 0400 and an ASA exposure index rating in the daylight of 100, and Ansco Triple S Pan.

Element 12 may be formed by applying to a suitable support 12a, for example, of baryta paper, a coating of a suspension or sol of the silica containing the silver precipitating agent. This sol is permitted to dry and provides layer 16. The suspension of silica may be obtained by dispersing the silica, for example, in water, and then adding the silver precipitating agent either directly or by introducing into the sol salts whose reaction product is the precipitating agent. The sol may also be applied to the sheet without the silver precipitating agent, and the sheet with the layer of silica thereon may then be dipped in a solution or mixture of the silver precipitating agent to deposit the latter in said layer.

When the foregoing liquid composition is spread or otherwise provided in a layer 14 between elements 10 and 12, the liquid thereof permeates the photosensitive layer 10b and the developing agent acts to develop the latent image in said layer. Almost simultaneously with the development, the complex-forming substance, i. e., sodium thiosulfate, forms a soluble silver complex with the undeveloped silver halide, and the silver complex is transported by the liquid of the processing agent to layer

16 of element 12. The presence of layer 16 results in a vigorous and relatively concentrated precipitation of the silver from the silver complex to form an image of improved density and color, and having more desirable gamma and contrast characteristics than would be obtained in the absence of the silica.

Examples of processes for forming a positive image wherein a silver halide transfer takes place and examples of the novel product of the invention which is used as the print-receiving element in the performance of said processes are given below, but it is expressly understood that these examples are merely illustrative and that the invention is not limited to the materials or proportions set out therein.

#### Example 1

A processing agent is prepared which comprises:

|                                   | Grams |
|-----------------------------------|-------|
| Water                             | 1860  |
| 20 Sodium carboxymethyl cellulose | 117   |
| Sodium sulfite                    | 78    |
| Sodium hydroxide                  | 74.6  |
| Sodium thiosulfate                | 14.5  |
| Citric acid                       | 38.5  |
| 25 Hydroquinone                   | 52    |

The processing agent is prepared by dissolving the sodium carboxymethyl cellulose, for example the commercially available Hercules 1362 medium viscosity type, in the water in a mixer at room temperature, and the solution is mixed therein for approximately one hour. Thereafter, the sodium sulfite, sodium hydroxide, sodium thiosulfate and citric acid are added to the solution, the addition being effected in an inert atmosphere, for example of nitrogen. Upon dissolution of these materials, the hydroquinone is added and the solution is further mixed for an hour at approximately room temperature in a non-oxidizing atmosphere of nitrogen.

A print-receiving element 12 provided with a silver precipitating stratum 16 is prepared by having at least 40 the baryta-coated surface portion of a strip of baryta paper immersed in a mixture comprising the following ingredients:

|                                                                                                                             |          |
|-----------------------------------------------------------------------------------------------------------------------------|----------|
| 1% solution of sodium sulfide                                                                                               | cc. 280  |
| Silica aerogel                                                                                                              | grams 30 |
| 45 Solution containing 30 g. sodium acetate, 1 g. neutral lead acetate and 30 g. zinc nitrate dissolved in 100 cc. of water | cc. 92   |

50 to provide a thin coating of these materials on said surface. As the baryta paper is removed from the bath, the excess mixture on said surface is removed from the sheet as, for example, by the action of a soft buffer roll on said sheet as it leaves the bath.

The processing agent is spread in a layer 14 of approximately .002-.003" in thickness between the coated surface of element 12 and the photosensitive silver halide emulsion 10b of a photosensitive film 10. Emulsion 10b is a relatively high-speed orthochromatic emulsion like the emulsion of Eastman Kodak Verichrome film, and has been exposed to predetermined subject matter to form therein a latent image of said subject matter, support 10a for said emulsion being a white paper. The laminations formed by the spreading of the processing agent in a layer 14 between elements 10 and 12 is kept intact for approximately one-half to one and one-half minutes, preferably one minute, and at the end of this time element 12 is stripped from element 10. Element 12, when so stripped, carries a positive print in silver of the subject matter of the latent image in emulsion 10b. The sodium carboxymethyl cellulose of layer 14 adheres to coating 16 of element 12 and solidifies to form a film thereon. The print obtained in this manner has good color, density and other pictorial qualities.

Other materials may be substituted for those used in the foregoing process and the proportions may be varied to an appreciable extent. For example, the film-forming material in the processing agent which imparts the desired viscosity to the latter may be any of the high molecular weight polymers which are stable to alkalies and which are soluble in aqueous alkaline solutions. For example, such other plastics as hydroxyethyl cellulose, polyvinyl alcohol and the sodium salts of polymethacrylic acid and polyacrylic acid may be used. The plastic is preferably contained in the agent in sufficient quantities to impart to the composition a viscosity in excess

of 1,000 centipoises at a temperature of approximately 24° C. Preferably, the viscosity of the processing agent is of the order of 1,000 to 200,000 centipoises.

Other developing agents may be used, for example one of the following: p-aminophenol hydrochloride; bromo-5-hydroquinone; chlorohydroquinone; diaminophenol hydrochloride; diaminophenol dihydrochloride; tolulydroquinone; monomethyl-p-aminophenol sulfate; a mixture consisting by weight of one-half hydroquinone and one-half p-hydroxyphenylaminoacetic acid; and a mixture consisting by weight of one-fourth hydroquinone and three-fourths p-hydroxyphenylaminoacetic acid.

To form the soluble silver complex, such other complex-forming substances as sodium thiocyanate, ammonium thiocyanate and ammonia may be employed.

Examples of further embodiments of the novel print-receiving elements of the present invention and the processes for forming the same are given below:

*Example 2*

To 24 cc. of a 10% solution of lanthanum chloride there is added 4 g. of silica aerogel (Santocel C) and 6 cc. of a 1% solution of sodium sulfide, and these ingredients are thoroughly mixed in a mechanical mixer. A layer of the resulting mixture is then applied to the baryta-coated surface of a sheet of baryta paper, and the sheet is permitted to stand for approximately 15 seconds. Thereafter, the excess of the liquid mixture is removed as by a soft buffer roll from the surface of the sheet.

*Example 3*

The process of forming the sheet described in Example 2 may be performed by substituting for the mixture therein a mixture of the following materials which gives a coating of silica containing palladium sulfide:

24 cc. of a 10% solution of palladium chloride  
4 g. of silica aerogel  
4 cc. of a 1% solution of sodium sulfide

*Example 4*

The process of forming the sheet described in Example 2 may be performed by substituting for the mixture therein a mixture of the following materials which gives a coating of silica containing nickelous sulfide:

40 cc. of a 15% solution of nickelous chloride  
7.5 g. of silica aerogel  
20 cc. of a 1% solution of sodium sulfide

*Example 5*

The process of forming the sheet described in Example 2 may be performed by substituting for the mixture therein a mixture of the following materials which gives a coating of silica containing cadmium sulfide:

96 cc. of a 20% solution of cadmium acetate  
15 g. of silica aerogel  
30 cc. of a 1% solution of sodium sulfide

*Example 6*

The process of forming the sheet described in Example 2 may be performed by substituting for the mixture therein a mixture of the following materials which gives a coating of silica containing zinc sulfide:

20 cc. of a 37.5% solution of zinc nitrate  
7.5 g. of silica aerogel  
30 cc. of a 1% solution of sodium sulfide

*Example 7*

The process of forming the sheet described in Example 2 may be performed by substituting for the mixture therein a mixture of the following materials which gives a coating of silica containing magnesium sulfide:

48 cc. of a 40% solution of magnesium acetate  
7.5 g. of silica aerogel  
18 cc. of a 1% solution of sodium sulfide

*Example 8*

The process of forming the sheet described in Example 2 may be performed by substituting for the mixture therein a mixture of the following materials which gives a coating of silica containing lead selenide:

96 cc. of a 40% neutral lead acetate solution  
15 g. of silica aerogel  
30 cc. of a 1% sodium selenide solution

*Example 9*

To 15 grams of Ludox, a solution containing approximately 30% of hydrated colloidal silica in water, there is added 90 grams of water. Thereafter 24 cc. of a solution formed by adding 3 grams of sodium sulfide to 46 cc. of water is added to this suspension, followed by the addition of 12 cc. of a solution formed by dissolving 2.6 grams of lead acetate in 20 cc. of water.

The resulting mixture is rubbed by hand on the surface of the print-receiving support. It is preferable to wipe off any excess of the mixture from the paper after the rubbing operation.

To obtain different precipitating agents in the silver precipitating layer that is formed according to the process of Example 9, there may be substituted for the 2.6 grams of lead acetate one of the following salts in the following quantities:

|                   | Grams |
|-------------------|-------|
| 20 Zinc acetate   | 1.42  |
| Cupric acetate    | 1.34  |
| Manganous acetate | 1.60  |
| Cadmium acetate   | 1.92  |

*Example 10*

A suspension is formed by mixing 20 grams of silica aerogel in 100 cc. of water. This sol or suspension is then rubbed onto the baryta-coated surface of a sheet of baryta paper. The sheet is then dried and dipped in a 3% water solution of sodium sulfide for thirty seconds. The excess liquid is squeegeed from the sheet as it is removed from the solution.

*Example 11*

35 A suspension is formed by mixing 20 grams of silica aerogel in 100 cc. of water. This sol or suspension is then rubbed onto the baryta-coated surface of a sheet of baryta paper. The sheet is then dried and dipped in a 3% water solution of sodium sulfide for thirty seconds.

40 The excess liquid is squeegeed from the sheet as it is removed from the solution. The sheet is then again dried and dipped for ten seconds in a second solution which is a 5% water solution of neutral lead acetate. The excess liquid is squeegeed from the surface of the sheet and the sheet is dried once more before being used.

*Example 12*

To assure the presence of a sufficient excess of cations for capturing the sulfide or selenide ions of any of the print-receiving elements 12 of the foregoing Examples 1 through 11, said elements may be suitably treated as follows: The surface of the element containing the silica suspension is dipped for 30 seconds in a solution consisting of:

55 10 grams cadmium acetate  
1 gram lead acetate  
30 grams zinc acetate  
100 cc. of water

Excess moisture is removed from the sheet as it leaves the solution, for example with a glass rod, and the sheet is dried.

For the baryta paper of any of the foregoing examples, there may be substituted a film of plastic such, for example, as polyvinyl alcohol, hydroxyethyl cellulose, sodium carboxymethyl cellulose, regenerated cellulose or other self-supporting sheetlike materials upon which the novel silver precipitating layer of the present invention may be deposited.

In another form of the product of the present invention, it may be desirable to provide a coating on the silver precipitating layer 16 of a material, such as a plastic, more abrasion-resistant than the silica of the precipitating layer in order to protect said layer. This overcoat of a plastic material may also serve as a layer which prevents the adhesion to the element 12 of the film-forming material of the layer of processing liquid 14 so that when said element 12 is stripped away from the photosensitive film 10 at the completion of the processing, the film-forming material remains attached to the photosensitive layer 10b.

An embodiment of a print-receiving element of this construction is shown in Fig. 3 wherein 12a is the support, 16 is the silver precipitating layer, both of which are like layers 12a and 16 of Fig. 1, and there is applied over layer 16 a thin coating of a film-forming material

## 11

18 which may be, for example, gum arabic, cellulose acetate-hydrogen phthalate, polyvinyl alcohol, hydroxyethyl cellulose, methyl cellulose, ethyl cellulose, cellulose nitrate, sodium alginate, pectin and polymethacrylic acid. Layer 18 preferably has a thickness of the order of 1-3 microns, although if it is relatively water permeable its thickness may be appreciably greater. Layer 18 may contain one or more of the neutralizing agents which tend to improve the stability of the finished print.

To provide any of the print-receiving elements 12 of Examples 1 through 12 with a protective coating 18 of a more abrasion-resistant plastic which may also serve as a layer for minimizing the adhesion between the film-forming material of layer 14, particularly where said material is sodium carboxymethyl cellulose, said elements 12 of each of said examples may be processed as follows:

## Example 13

The processed sheet has roll coated thereon against a smooth surface such, for example, as the polished surface of a metal drum, a 5% aqueous solution of polyvinyl alcohol in a layer whose thickness is of the order of .001 inch. An equivalent amount by weight of hydroxyethyl cellulose or polymethacrylic acid may be substituted for the polyvinyl alcohol of this example.

## Example 14

The processed sheet is dipped into a 2% solution of cellulose acetate, the cellulose acetate being dissolved in a mixture of methanol, ethyl acetate and methyl cellosolve, the proportions of said solvents being in the ratio of 1:3:3 by volume, respectively. The dipped baryta paper is removed from the solution in a vertical position to permit the excess liquid to drip off, a sufficient quantity of the solution remaining on the surface of the paper to provide the latter with a coating of cellulose acetate of the desired thickness.

## Example 15

A 10% solution of cellulose acetate-hydrogen phthalate in acetone is roll coated on the processed sheet in a thickness of approximately .001 inch.

In a similar manner, such other materials as methyl cellulose, cellulose nitrate, sodium alginate, ethyl cellulose, gum arabic and pectin may be applied as layer 18 to the processed sheet. It is, of course, understood that suitable solvents for the materials are employed, said solvents being preferably water for such materials as are readily water soluble, and may be toluene for ethyl cellulose and a mixture of methanol and ethyl acetate for cellulose nitrate.

Although the silver precipitating layer of the present invention is constituted primarily of the silica, it may contain therein a small quantity, preferably not exceeding 10% by weight of the silica, of a film-forming substance such as gum arabic, hydroxyethyl cellulose or any of the other materials heretofore mentioned as being suitable for the abrasion-resistant coating 18 on layer 16. The addition of this small quantity of plastic facilitates application of the layer 16 onto the support theretofore. An example of one way of forming a layer 16 containing a small quantity of film-forming material is the following:

## Example 16

The following ingredients are mixed in the order named:

|                 |       |       |
|-----------------|-------|-------|
| Water           | cc    | 595   |
| Gum arabic      | cc    | 3.5   |
| Cadmium acetate | grams | 22.76 |
| Silica aerogel  | do    | 36    |
| Sodium selenide | do    | 10    |

A sheet of baryta is dipped in the mixture, withdrawn, and the excess liquid squeezed therefrom.

Other plastics may be substituted for the gum arabic. Also, by substituting salts of other metals for the cadmium acetate different metallic selenides may be obtained in the sol.

Another class of compounds especially useful in controlling the alkalinity of the print-receiving element after the formation of the positive print therein is the organic compounds which react in alkaline solution to consume alkali, as disclosed in my above-noted U. S. Patent No. 2,635,048. Preferred from this class are the esters (including lactones), the anhydrides, the alpha-halohydrins

and the aldehydes which have a specific rate of alkaline hydrolysis at 25° C. greater than 80 liters per mol per minute and, from this class, the preferred species are compounds which do not volatilize too rapidly, i. e., compounds whose boiling points are in excess of 150° C.

Examples of preferred species of these compounds are: diethyl oxalate, ethyl oxamate, diethyl d-tartrate, a hydroxybenzaldehyde, dimethyl diacetyltartrate, dimethyl fumarate, dimethyl malate, dimethyl oxalate, dimethyl tartrate, polyethylene oxalate, benzoic anhydride, di-n-butyl oxalate, n-butyl oxamate, di-n-butyl tartrate, trimethyl citrate, ethyl cyanoacetate, ethyl N-B hydroxyethyl oxamate, glucono delta lactone, glyceryl trimethyl oxalate and cellulose methyl oxalate, di-B-hydroxyethyl malonate, hydroxyethyl lactate, diethyl malate, diethyl tartrate, di-B-hydroxyethyl malate, ethyl acetoacetate, diethyl malate, butyl lactate, diethyl malonate, glyceryl chlorohydrin, and di-B-hydroxyethyl succinate.

The positive print is subject to several sources of instability which stem, for example, from the oxidation of the developer in the highlights, the discoloration of some of the unexhausted chemical components in the positive prints by exposure to visible and near visible radiation, and the partial bleaching of the silver.

It has been determined that these effects are most nearly eliminated by combining the stabilizing effects of the soluble metallic salts and the organic alkali-consuming compounds, i. e., by using at least one of each of these classes of stabilizers in the print-receiving element.

Examples of suitable print-receiving elements which embody this combination of stabilizers, together with the novel silver precipitating layer of the invention, are the following:

## Example 17

The baryta-coated surface of a sheet of baryta paper is immersed in a mixture consisting of:

|                     |       |      |
|---------------------|-------|------|
| Water               | cc    | 1000 |
| Arabol              | cc    | 150  |
| Dimethyl d-tartrate | grams | 400  |
| Lead acetate        | do    | 70   |
| Cadmium acetate     | do    | 50   |
| Zinc acetate        | do    | 40   |

The sheet is then dried and there is applied over the foregoing coating a further coating consisting of:

|                                    |       |      |
|------------------------------------|-------|------|
| Silica aerogel                     | grams | 300  |
| 1% aqueous solution sodium sulfide | cc    | 2800 |
| Cadmium acetate                    | grams | 30   |
| Lead acetate                       | do    | 1    |
| Zinc nitrate                       | do    | 30   |
| Water                              | cc    | 100  |

## Example 18

The baryta-coated surface of a sheet of baryta paper is dipped in a solution consisting of:

|               |       |      |
|---------------|-------|------|
| Ethanol       | cc    | 1000 |
| Zinc nitrate  | grams | 120  |
| Ethyl oxamate | do    | 90   |

The treated surface of this sheet is then provided with a sulfide-containing coating consisting of the following:

|                                    |       |      |
|------------------------------------|-------|------|
| Silica aerogel                     | grams | 300  |
| 1% aqueous solution sodium sulfide | cc    | 2800 |
| Cadmium acetate                    | grams | 30   |
| Lead acetate                       | do    | 1    |
| Zinc nitrate                       | do    | 30   |
| Water                              | cc    | 100  |

It is to be noted from the foregoing examples that the silver precipitating agent is present in the sheet in a very small amount. Concentrations, for example, as low as  $2 \times 10^{-6}$  to  $2 \times 10^{-5}$  gram-moles for each square foot of the surface area of the print-receiving element have proven adequate.

Since certain changes may be made in the above product and process without departing from the scope of the invention herein involved, it is intended that all matter contained in the above description or shown in the accompanying drawing shall be interpreted as illustrative and not in a limiting sense.

What is claimed is:

1. A photographic product comprising a photosensitive material which includes a silver halide layer, a base layer having adjacent one surface thereof a silver precipitating stratum, said stratum comprising a silver

precipitating agent dispersed among colloidal particles of silica, and a rupturable containing means holding a liquid, said product having positioned therein photographic reagents, including a silver halide developer and a silver halide solvent, said containing means and said layers being so held together that said containing means is capable, upon rupture, of releasing at least a part of its contents to permeate superposed portions of said silver halide layer and said base layer, said liquid, upon release, rendering said silver halide developer and said silver halide solvent effective to develop a latent image in said silver halide layer and to form soluble silver complex with the undeveloped silver halide of said silver halide layer, said liquid, upon release, additionally transporting said soluble silver complex in the direction of said silver precipitating agent wherein part at least of the soluble silver complex is reduced to silver to produce the positive print.

2. A photographic product comprising a silver halide layer, a base layer and a rupturable container holding a liquid, said layers and said container being attached together so as to permit said layers to be superposed with said container so positioned as to release its liquid for spreading in a film between said layers, the liquid in said container comprising a silver halide developer, a silver halide solvent and a thickening agent, said base layer having adjacent one surface thereof a stratum including a silver precipitating agent dispersed among colloidal particles of silica.

3. A photographic product capable of forming transfer prints in conjunction with a photosensitive silver halide element, said product comprising a rupturable containing means, holding a liquid, and a sheet support upon which said containing means is mounted, said sheet support providing an image-receiving area adjacent said containing means onto which said liquid is spreadable in a thin layer directly from said containing means, said product carrying a silver halide developer and a silver halide solvent, said sheet support having, adjacent the surface mounting said containing means and at least coextensive with said image-receiving area, a silver precipitating stratum comprising a silver precipitating agent dispersed among colloidal particles of silica, said silver halide developer, said silver halide solvent and said liquid being sufficient in amount and being so located, in relation to said image-receiving area, that the spreading of said liquid over said area disperses silver halide developer and silver halide solvent throughout said area in adequate quantity to form a transfer print of a latent image in an area of a contiguous silver halide element equivalent to said image-receiving area.

4. A photographic product capable of forming transfer prints in conjunction with a photosensitive silver halide element, said product comprising a rupturable containing means, holding an alkaline liquid solution of a silver halide developer, a silver halide solvent and a film-forming plastic, and a sheet support upon which said containing means is mounted, said sheet support providing an image-receiving area adjacent said containing means onto which said liquid solution is spreadable in a thin layer directly from said containing means, said support having a silver precipitating stratum at least coextensive in area with said image-receiving area, said silver precipitating stratum comprising a silver precipitating agent dispersed among colloidal particles of silica, said solution and the silver precipitating agent in said stratum being sufficient in amount so that the spreading of said liquid over said image-receiving area provides a dispersion of silver halide developer and silver halide solvent in adequate quantity to form a transfer print of a latent image in an area of a contiguous silver halide element equivalent to said image-receiving area.

5. The process of forming positive images in silver which comprises developing a latent negative image in a silver halide emulsion layer with a solution comprising a silver halide developer and a silver halide solvent to form an imagewise distribution of soluble silver complex in said emulsion layer, transferring from said emulsion layer by imbibition at least part of said imagewise distribution of said soluble silver complex to an image-carrying layer comprising a support and an image receiving stratum so superposed adjacent said emulsion layer as to

receive a depthwise diffusion of said solution from said emulsion layer without appreciably disturbing the imagewise distribution of the silver complex in said solution, said stratum comprising a distinct and separately applied coating of colloidal silica on said support and including a silver precipitating agent dispersed in said coating, and reducing to silver the silver ions of said soluble silver complex in said stratum to form an image in silver among colloidal particles of said silica which is a positive of the subject matter of said latent image.

6. A print-receiving element for having transfer prints formed thereon by precipitating the silver of an imagewise distribution of a soluble silver complex brought into contact therewith, said element comprising a support and a silver precipitating layer, at least one surface portion of said element, including said layer, being permeable to an aqueous solution of a soluble silver complex, said layer comprising a silver precipitating agent finely dispersed among colloidal particles of silica, said support for the silver precipitating layer comprising a sheet of baryta paper, said silver precipitating agent being at least one substance from the class consisting of heavy metals, metal sulfides and selenides, and organic thio compounds.

7. A print-receiving element for having transfer prints formed thereon by precipitating the silver of an imagewise distribution of a soluble silver complex brought into contact therewith, said element comprising a support and a silver precipitating layer, at least one surface portion of said element, including said layer, being permeable to an aqueous solution of a soluble silver complex, said layer being a distinct and separately applied coating on said support and comprising a silver precipitating agent finely dispersed among colloidal particles of silica, said silver precipitating agent being at least one substance from the class consisting of heavy metals, metal sulfides and selenides, and organic thio compounds and being present in a concentration of the order of  $2 \times 10^{-5}$  gram-moles for each square foot of the surface area of said layer.

8. A photographic product comprising a photosensitive material which includes a silver halide layer, a base layer having adjacent one surface thereof a silver precipitating stratum, said stratum comprising a matrix of submacroscopic discrete particles of silica and a silver precipitating agent dispersed in said matrix, and a rupturable containing means holding a liquid, said product having positioned therein photographic reagents, including a silver halide developer and a silver halide solvent, said containing means and said layers being so held together that said containing means is capable, upon rupture, of releasing at least a part of its contents to permeate superposed portions of said silver halide layer and said base layer, said liquid, upon release, rendering said silver halide developer and said silver halide solvent effective to develop a latent image in said silver halide layer and to form soluble silver complex with the undeveloped silver halide of said silver halide layer, said liquid, upon release, additionally transporting said soluble silver complex in the direction of said silver precipitating agent wherein part at least of the soluble silver complex is reduced to silver to produce the positive print.

9. A photographic product comprising a silver halide layer, a base layer and a rupturable container holding a liquid, said layers and said container being attached together so as to permit said layers to be superposed with said container so positioned as to release its liquid for spreading in a film between said layers, the liquid in said container comprising a silver halide developer, a silver halide solvent and a thickening agent, said base layer comprising a non-siliceous support and having adjacent one surface thereof a stratum including a silver precipitating agent dispersed among submacroscopic particles of silica which on the average are not smaller than colloidal in size.

10. A photographic product capable of forming transfer prints in conjunction with a photosensitive silver halide element, said product comprising a rupturable containing means holding a liquid, and a sheet support upon which said containing means is mounted, said sheet support providing an image-receiving area adjacent said containing means onto which said liquid is spreadable in a thin layer directly from said containing means, said product carrying a silver halide developer and a silver halide solvent, said sheet support having, adjacent the surface

mounting said containing means and at least coextensive with said image-receiving area, a silver precipitating stratum comprising a matrix of submacroscopic discrete particles of silica and a silver precipitating agent dispersed in said matrix, said silver halide developer, said silver halide solvent and said liquid being sufficient in amount and being so located, in relation to said image-receiving area, that the spreading of said liquid over said area disperses silver halide developer and silver halide solvent throughout said area in adequate quantity to form a transfer print of a latent image in an area of a contiguous silver halide element equivalent to said image-receiving area.

11. A photographic product capable of forming transfer prints in conjunction with a photosensitive silver halide element, said product comprising a rupturable containing means holding an alkaline liquid solution of a silver halide developer, a silver halide solvent and a film-forming plastic, and a sheet support upon which said containing means is mounted, said sheet support providing an image-receiving area adjacent said containing means onto which said liquid solution is spreadable in a thin layer directly from said containing means, said support having a silver precipitating stratum at least coextensive in area with said image-receiving area coated on a non-siliceous sheet, said silver precipitating stratum comprising a silver precipitating agent dispersed among submacroscopic particles of silica which on the average are not smaller than colloidal in size, said solution and the silver precipitating agent in said stratum being sufficient in amount so that the spreading of said liquid over said image-receiving area provides a dispersion of silver halide developer and silver halide solvent in adequate quantity to form a transfer print of a latent image in an area of a contiguous silver halide element equivalent to said image-receiving area.

12. The process of forming positive images in silver which comprises developing a latent negative image in a silver halide layer, reacting a silver halide solvent with part at least of the undeveloped silver halide of said layer to form an imagewise distribution of soluble silver complex in said layer, transferring in solution at least part of said imagewise distribution of said soluble silver complex to an image-receiving material comprising a support and a distinct and separately applied coating of submacroscopic, discrete particles of silica on said support and so located in relation to said silver halide layer as to receive the solution of said complex without appreciably disturbing its imagewise distribution, said coating having a silver precipitating agent dispersed among said silica particles, and reducing to silver the silver ions of said soluble silver complex at said image-receiving material to form an image in silver.

13. The process of claim 12 wherein said support is a flexible sheet support.

14. The process of claim 13 wherein said sheet support is paper.

15. The process of claim 13 wherein said sheet support is a sheet of transparent plastic.

16. The process of claim 12 wherein said silver precipitating agent is from the class consisting of heavy metals, metal sulfides and selenides, and organic thio compounds.

17. The process of forming positive images in silver which comprises developing a latent negative image in a silver halide emulsion layer with a solution comprising a silver halide developer and a silver halide solvent to form an imagewise distribution of soluble silver complex in said emulsion layer, transferring from said emulsion layer by imbibition at least part of said imagewise distribution of said soluble silver complex to an image-carrying element comprising a support and a distinct and separately applied coating of submacroscopic particles of silica at least colloidal in size and so superposed adjacent said emulsion layer as to receive a depthwise diffusion of said solution from said emulsion layer without appreciably disturbing the imagewise distribution of the silver complex in said solution, said coating having a silver precipitating agent dispersed among said particles of silica, and reducing to silver the silver ions of said soluble silver complex in said coating to form an image in silver among said particles of silica.

18. The process of claim 17 wherein said particles of silica form a macroscopically continuous matrix for said

precipitating agent and said matrix is a coating on a flexible sheet support.

19. The process of claim 18 wherein said sheet support is a sheet of paper.

20. The process of claim 18 wherein the sheet support is a sheet of transparent plastic.

21. The process of claim 17 wherein said silver precipitating agent is from the class consisting of heavy metals, metal sulfides and selenides, and organic thio compounds.

22. The process of claim 17 wherein said silver precipitating agent is a colloidal heavy metal.

23. The process of claim 17 wherein said silver precipitating agent is a colloidal noble metal.

24. The process of claim 17 wherein said silver precipitating agent is at least one compound from the class consisting of the heavy metal sulfides and selenides.

25. The process of claim 17 wherein said silver precipitating agent is an organic thio compound.

26. A print-receiving element for having transfer prints formed thereon by precipitating the silver of a soluble silver complex brought into contact therewith, said element comprising a support and a substantially non-photosensitive silver precipitating layer provided as a discrete macroscopically continuous, distinct and separately applied coating on one surface of said support, one surface portion of said element including said layer being permeable to an aqueous solution of a soluble silver complex, said layer having a major proportion by weight of submacroscopic particles of silica on the average at least colloidal in size and having finely dispersed therethrough a minor proportion by weight of particles of a silver precipitating agent for aiding the reduction and precipitation of metallic silver from silver complex ions in the presence of a reducing agent, said silver precipitating agent being from the class consisting of heavy metals, metal sulfides and selenides, and organic thio compounds.

27. A print-receiving element for having transfer prints formed thereon by precipitating the silver of a soluble silver complex brought into contact therewith, said element comprising a support and a substantially non-photosensitive silver precipitating layer provided as a discrete macroscopically continuous, distinct and separately applied coating on one surface of said support, one surface portion of said element including said layer being permeable to an aqueous solution of a soluble silver complex, said layer having a major proportion by weight of colloidal particles of substantially pure silica and having finely dispersed therethrough a substantially lesser amount by weight of particles of a silver precipitating agent for aiding the reduction and precipitation of metallic silver from silver complex ions in the presence of a reducing agent, said silver precipitating agent being from the class consisting of heavy metals, metal sulfides and selenides, and organic thio compounds.

28. A print-receiving element for having transfer prints formed thereon by precipitating the silver of a soluble silver complex brought into contact therewith, said element comprising a non-siliceous support and a substantially non-photosensitive silver precipitating layer provided as a discrete macroscopically continuous, distinct and separately applied coating on one surface of said support, one surface portion of said element including said layer being permeable to an aqueous solution of a soluble silver complex, said layer having a major proportion by weight of submacroscopic particles of silica aerogel and having finely dispersed therethrough a substantially lesser amount by weight of particles of a silver precipitating agent for aiding the reduction and precipitation of metallic silver from silver complex ions in the presence of a reducing agent, said silver precipitating agent being from the class consisting of heavy metals, metal sulfides and selenides, and organic thio compounds.

29. The product of claim 26 wherein said silver precipitating agent is a colloidal heavy metal.

30. The product of claim 26 wherein the silver precipitating agent is a compound from the class consisting of the heavy metal sulfides and selenides.

31. The product of claim 26 wherein said silver precipitating agent is an organic thio compound.

17

## References Cited in the file of this patent

## UNITED STATES PATENTS

| Number    | Name    | Date           | Number  |
|-----------|---------|----------------|---------|
| 2,296,636 | Hanahan | Sept. 22, 1942 | 358,672 |
| 2,352,014 | Rott    | June 20, 1944  | 873,507 |
| 2,626,867 | Webster | Jan. 27, 1953  | 59,365  |

18

## FOREIGN PATENTS

| Country       | Date          |
|---------------|---------------|
| Great Britain | Oct. 15, 1931 |
| France        | Mar. 23, 1942 |
| Netherlands   | May 16, 1947  |

## OTHER REFERENCES

10 Burmistrov, Photographic Journal, vol. 60, August 1936, pp. 452-459.